

F. E. IVES,  
COLOR PHOTOGRAPHY,  
APPLICATION FILED DEC. 5, 1912.

1,173,429.

Patented Feb. 29, 1916.

*Fig. 1.*



*Fig. 2.*

Attest:

J. D. Mitchell

E. B. King

Inventor:

Frederic E. Ives,  
by Rogers, Kennedy & Campbell,  
his Atty's.

# UNITED STATES PATENT OFFICE.

FREDERIC E. IVES, OF WOODCLIFFE-ON-HUDSON, NEW JERSEY.

## COLOR PHOTOGRAPHY.

1,173,429.

Specification of Letters Patent. Patented Feb. 29, 1916.

Application filed December 5, 1912. Serial No. 735,064.

To all whom it may concern:

Be it known that I, FREDERIC EUGENE Ives, a citizen of the United States, residing at Woodcliff-on-Hudson, in the county of Bergen and State of New Jersey, have invented certain new and useful Improvements in Color Photography, of which the following is a specification, reference being had therein to the accompanying drawing.

10 My invention relates to the art of color-photography and more particularly to a novel color-photography plate-pack and to a method of making the same.

While the present improvement might be applicable in connection with color-photography in two colors or in four colors, it is particularly intended for the three-color system, and is more especially directed to the red-sensitive and green-sensitive elements used therein.

An example of a plate-pack for the trichromatic or three-color system of color-photography is illustrated in my Patent No. 927,244, of July 6, 1909, in which the red-sensitive member or plate and the green-sensitive member or film are used pressed together in face contact, so that light rays passing from the objective of the camera through one of the transparent plates or 20 films forms an image upon both of the closely contacting sensitive coatings thereof, thus making by a single exposure both a red and green photographic record, as required in the trichromatic process. Possibly the principles hereof would be applicable to contacting sensitive plates for other than the green and red light components of the image, and in any case the plate-pack and arrangement of my Patent 980,961 of 30 Jan. 10, 1911 could be used for carrying out the present improvements.

I will endeavor to first state the conditions in which has arisen the problem which I have met by the present invention. Photographic plates of the usual or silver bromid species can be prepared which are sensitive to green and not to red light, but it is not known how to prepare plates which will be sensitive to red light without being 40 sensitive to some extent also to green light. For this reason the green-sensitive plate may be placed at the front and a red coating interposed between the two plates preferably on the surface of the green-sensitive plate, such coating being entirely superficial and extremely tenuous and water soluble, its

presence serving to prevent any substantial amount of green light from reaching the red-sensitive plate. The tenuous and temporary intermediate color coating is therefore 60 one of the important requisites of a plate-pack such as the present improvements relate to.

A further requirement for attaining perfection in such a plate-pack is that the red-sensitive and green-sensitive plates shall have substantially identical gradation-giving qualities, and also density-giving qualities. This requirement cannot be insured, and it is rarely if ever possible when the red 65 and green-sensitive plates are either manufactured in different factories or by different processes or even when made from different batches of emulsion in the same factory. In all those cases the qualities referred to usually vary quite measurably and materially, even as between emulsions made by the same formula at the same factory at different times. If the said requirement is attempted to be attained, or the said difficulty minimized, by taking ordinary sensitive plates, all from a single batch, and sensitizing half of them for red, and half of them for green, by the usual processes of bathing in suitable color-sensitizing dyes, 70 practical satisfaction is impossible. One reason for this fact is that no known sensitizing dyes which sensitize for green but not red will produce satisfactory plates of 75 high speed and good keeping quality unless 80 the dyes be added to the emulsion before the plates are coated, in which case the entire batch is green-sensitive.

The principal part of the present improvement is that by which I have solved 95 the difficulties and attained the requirements referred to, thus making available green-sensitive and red-sensitive plates of uniformly and reliably equal qualities, which when placed face to face in a plate-pack will 100 give results for color-photography of the highest satisfaction.

It must be appreciated that in the trichromatic system of color-photography, the process is one of analysis or separation of 105 the three elemental color components of the image, and that consequently the perfection of the finished picture must depend upon the true preservation of the relative density and gradation of color in all of the 110 three component color records. Reference has been made principally to the red and

green components, and the third component is the blue, as to which the same difficulties do not pertain that exist in the cases of the red and green records. Thus in my prior 5 patent No. 927,244, the blue-sensitive plate is placed at the front of the contacting red and green ones, and is comparatively tenuous and transparent, and either uncolored or else colored in such way as to assist the 10 proper formation of the red and green records.

Another feature of the present improvements comprises an improved method of obtaining a red superficial color layer over the 15 green-sensitive film.

A third feature of the present improvements resides in perfecting the same through an opaque backing to the rearmost or red-sensitive plate, for the purposes and 20 in the manner hereinafter set forth.

Having referred generally to the nature of the present improvements and the difficulties to be overcome, I will now refer more specifically to the preferred details in a 25 method of carrying out the invention.

I have made the discovery that the iso-cyanin red-sensitizing dyes are extremely prepotent over the fluorescein green-sensitizing dyes, so much so in fact that plates 30 made green-sensitive, for example, by the addition of eosin to the emulsion may afterward be bathed for from under a minute to several minutes in a weak solution of pinachrome or of pinacyanol, or a mixture of 35 the two, and thereby rendered red-sensitive; and that moreover red-sensitive plates so produced will be substantially identical in character with plates originally sensitized for the red rays by the dye solutions last 40 mentioned. By the employment of this discovery I am enabled to secure a perfectly true and reliable set of plates, or a plate-pack, in which the red and green-sensitive plates will have the same qualities as to 45 gradation and density. I prefer to proceed as follows. Commencing with a stock of green-sensitive plates all produced from the same emulsion containing a fluorescein green-sensitizing dye, or the equivalent, I 50 divide the same into two equal lots. One such lot of plates will then be converted and rendered red-sensitive by treatment in the pinachrome or pinacyanol solution. The two elements of the pack are thus made alike 55 in age and speed, and in density- and gradation-giving qualities. When I say "color sensitizing" or similar expression, it will be understood that I use the term in the ordinary sense of giving to a sensitive plate a 60 sensitiveness for a particular color or colors. The usual silver bromid plate may be described as a blue-sensitive plate for the reason that its original sensitiveness is such that the action of blue light very greatly 65 preponderates over that of other colors.

But if we treat the emulsion from which such a plate is made, or the plate itself, with certain dye-sensitizing agents for green, we in reality have a plate which is sensitive to both blue and green, but this is spoken of as 70 a green-sensitive, or more correctly, a green-sensitized plate. A yellow screen eliminates the blue rays. If the green sensitized plate be converted according hereto, or red-sensitized, it will be sensitive to blue, green and 75 red, the yellow and red screens, however, eliminating the blue and green rays. A red-sensitive plate, therefore, is not sensitive only for red, but is red-sensitized, permitting other colors to be screened out, and 80 enabling a true color-record of red rays to be secured. It should be further explained that a dye-sensitizer for green does not mean a green dye, as on the contrary it will probably have actually a minus-green color. 85

We now have the green-sensitive and red-sensitive elements of the plate set or pack. Before assembling the plates in pairs for making up the plate-packs, the second lot will be coated with the temporary screen 90 coating for shutting out the green rays from the adjacent red-sensitive plate. Upon assemblage in pairs, the plate-packs are complete except so far as blue-sensitive plate is to be combined or employed in conjunction 95 therewith.

I have above referred to the interposition upon the green-sensitive layer of a temporary or water-soluble dye coating, and this may be accomplished substantially by the 100 method described in the aforesaid Patent 927,244, wherein an alcoholic solution of a suitable dye was flowed over the face of the plate. I prefer, however, the following described improved method by which I am 105 enabled to obtain a more even and more deeply colored coating. This improvement consists in adding to the alcoholic dye solution before the plate is coated, some ether and also a very small amount of soluble gun 110 cotton, after which the plate may be coated as before. With these additions the dye solution is of a practically more viscous character, but, what is very important, the ultimate thickness of the screen coating is 115 not measurably added to. Specifically this part of my invention may be practised by taking, for example, four ounces of alcohol and two ounces of ether, saturated with a suitable dye such as fuchsin and adding 120 one grain only of soluble gun cotton. By this formula is obtained an even and deeply colored, but quite superficial and immeasurably thin coating of water-soluble dye, in the use of which there will be probably not 125 more than two thousandths of a grain of soluble gun cotton deposited upon each square inch of surface, leaving it freely water permeable.

We now have a plate-pack comprising 130

a red-sensitive plate face to face with a green-sensitive plate which is red-coated. Such an assemblage is, especially upon the red-sensitive plate, susceptible to halation 5 and also to injury by accidental exposure to light during handling, in use, and while making up the plate-packs. To prevent this and to perfect the plate-pack hereof to the farthest degree, I provide the red-sensitive plates with a backing which is opaque 10 to red light and which is in optical contact with the glass on the side opposite to the red-sensitive film. This efficiently avoids the dangers referred to. There would be a difficulty in applying the backing after the 15 plates are made red-sensitive, because they are unable to be exposed to much light of any kind, so that the necessary steps are hindered. I, however, propose herein to apply a backing by the aid of red illumination 20 and at a time before the plates are made red-sensitive, which I find can be readily and satisfactorily accomplished if the present invention is employed. Light-excluding 25 backings as are already known, such for example as colored collodion or gum containing lampblack, are not suitable because either the color or the substance itself is liable to be partly dissolved in the subsequent 30 color-sensitizing solution, to the injury of the solution or the backing or both. I have overcome these difficulties and solved the problems stated, by employing for the backing of the red-sensitive plate a solution 35 of asphaltum in benzol, in which a quantity of some suitable oil-soluble blue dye is dissolved. This solution is easily applied by a brush or by flowing over the plate, and it dries very quickly, and when dry is insoluble 40 in the color sensitizing bath which is made up of dye, water and alcohol. Blue is selected as a suitable minus-red color.

The complete formula may be: benzol 28 oz., bitumen 3 oz., Hoechst Company's 45 oil soluble blue dye  $1\frac{1}{2}$  oz. With some qualities of bitumen it may be advantageous to replace 3 ozs. or 4 ozs. of the benzol with the same quantity of sulfuric ether.

I will now sum up completely the steps 50 involved in the present invention. We first produce a batch of green-sensitive plates preferably by use of the specific chemical or dye mentioned. Or we otherwise procure them, they being an ordinary commodity on the market. This batch of plates is then 55 divided into two parts. Taking the first portion of the plates, they will first be coated at the back with the specific opaque coating referred to, which will be allowed to dry, 60 and the plates will then be treated for rendering them red-sensitive, preferably by the use of the specific dyes hereinabove named, dissolved in a mixture of alcohol and water. In the meantime, the second 65 portion of the plates which are already

green-sensitive, will be superficially coated with a temporary screen, such for example as the red colored screen specifically referred to hereinabove. Having our two components we assemble them to form a plate- 70 pack, and if desired combine a blue-sensitive plate therewith, for example by locating the same in front of the green-sensitive plate. By then securing the whole together, we have a unitary and easily handled plate- 75 pack which may be exposed in any desired manner. There for example may be a single exposure in an ordinary camera, as set forth in said prior Patent 927,244. After exposure the plates will be separated and 80 developed and fixed. Finally the opaque backing upon the red-color record or negative can be easily removed by means of a piece of cloth moistened with benzol or turpentine, and the three negatives or color-records are 85 ready for the subsequent steps of making the prints or positives.

The chemical or dye which gives a plate sensitiveness for a given color may be termed a color-sensitizing agent, and the plate a 90 dye-sensitized plate. The green-sensitizing agent already named, is preferably included in the original emulsion, and is so used in the complete and preferred embodiment of this invention. When I refer to a sensitive 95 plate, it is understood that as a carrier either a rigid glass plate or a flexible film is included.

As the physical arrangement of the components of the plate-pack hereof is susceptible of illustration, I have shown the same in the accompanying drawing, in which Fig. 1 shows a partial cross-section taken transversely of the plane of the plate-pack, 100 with the several members or components 105 slightly separated for clearness. Fig. 2 shows certain modifications.

In the figures the plate-pack 1 is shown as consisting of a plurality of members, 110 namely the three members 2, 3 and 4, which beginning from the rear may be made up as follows.

The member 2 at the rear has the opaque back screen 5 of the composition and applied in the manner specified, upon the rear surface of the carrier or glass plate 6, at whose front face is the red-sensitive coating 7 produced as before described, by a conversion from green-sensitiveness.

The plate-pack member 3 may be made 120 up, as shown in Fig. 1, of a red color-screen 8, of the composition previously stated, applied superficially upon the rear side of the green-sensitive coating 9, carried upon the carrier 10, which may be a thin transparent 125 film as in prior patent 927,244.

The plate-pack member 4, if a third member be employed, may be made up of a yellow color-screen 11 superficially spread over a blue-sensitive coating 12 upon a carrier or

glass plate 13, as shown, provided that member 3 has a thin transparent film, and all are secured together as in patent 927,244.

The three members 2, 3 and 4 constituting 5 the plate-pack 1 may be secured together in the manner of my prior patent 927,244, or the red and green-sensitive plates may be at one point and the blue-sensitive at another point in such a camera as that of my 10 prior patent 980,961, or the red and green plates might even be exposed at separated points, and the advantages of equal density and gradation are obtained. Obviously 15 many variations in the specific make-up of the pack might be introduced; for example, the color-screen 8 might be, as shown in Fig. 2, upon the coating 7 rather than the coating 9, or the color-screen 11 might be as in Fig. 2 omitted from the coating 12; 20 or the carrier 10 might be of thin film or of glass at will, glass being preferred when the member 4 is omitted from the pack; or the described arrangement might be employed in connection with different color- 25 sensitiveness for members 2 and 3.

It will thus be seen that I have described a plate-pack and process which accomplish the objects and advantages hereinbefore recited, and other advantages will be apparent 30 to those practising the improvements.

Since various features and details hereof may be altered without departing from the main principles involved, I do not wish to be limited thereto excepting as set forth in 35 the appended claims.

What I claim and desire to obtain by Letters Patent is:

1. In the art of color photography the 40 process of producing a set of color selection negatives which comprises the following steps: treating one of a batch of photographic plates which have been previously sensitized for a certain color to convert it to sensitiveness for a different color, and simultaneously exposing such converted plate and an unconverted plate from the same batch to the same light image.

2. In the art of color photography the 50 process of producing a set of color selection negatives which comprises the following steps: treating one of a batch of photographic plates which have been previously sensitized for a certain color to convert it to sensitiveness for a different color, placing such converted plate face to face with an unconverted plate from the same batch, and simultaneously exposing said plates to the same light image.

3. In the art of color photography the 60 process of producing a set of color selection negatives which comprises the following steps: treating one of a batch of photographic plates which have been previously sensitized for a certain color to convert it to sensitiveness for a different color, secur-

ing together in face to face contact such converted plate with an uncovered plate from the same batch, and simultaneously exposing the two plates through the support of one of them.

4. In the art of color photography the process of producing a set of color selection negatives which comprises the following steps: treating one of a batch of photographic plates which have been previously sensitized for a certain color to convert it to sensitiveness for a different color prior to combining it with an unconverted plate from the same batch, applying a temporary superficial color screen upon the sensitive coating of one of said two plates, subsequently combining said two plates in face to face contact, and thereafter simultaneously exposing the combined plates to the same light image.

5. In the art of color photography the process of producing a set of color selection negatives which comprises the following steps: treating one of a batch of green sensitized photographic plates to convert it to red sensitiveness, and simultaneously exposing such converted plate and an unconverted plate from the same batch to the same light image.

6. In the art of color photography the 95 process of producing a set of color selection negatives which comprises the following steps: treating one of a batch of green sensitized photographic plates to convert it to red sensitiveness, securing together in face to face contact such converted plate with an unconverted plate from the same batch, and simultaneously exposing the two plates through the support of one of them.

7. In the art of color photography the 105 process of producing a set of color selection negatives which comprises the following steps: treating one of a batch of green sensitized photographic plates to convert it to red sensitiveness, placing such converted plate face to face with an unconverted plate from the same batch and with a transparent blue sensitive plate in front of both, and simultaneously exposing such three plates to the same light image.

8. In the art of color photography the process of producing a set of color selection negatives which comprises the following steps: preparing a batch of green sensitive photographic plates by incorporating a 120 fluorescein dye in the emulsion, treating one of such batch of plates to convert it to red sensitiveness by a prepotent color-selecting agent, and simultaneously exposing such converted plate and an unconverted plate 125 from the same batch to the same light image.

9. In the art of color photography the process of producing a set of color selection negatives which comprises the following 130

70

75

85

90

95

100

105

110

115

120

125

130

steps: preparing a batch of green sensitive photographic plates by incorporating a fluorescin dye in the emulsion, treating one of such batch of plates to convert it to red sensitiveness by an isocyanin dye, and simultaneously exposing such converted plate and an unconverted plate from the same batch to the same light image.

10. In the art of color photography the process of producing a set of color selection negatives which comprises the following steps: preparing a batch of green sensitive photographic plates by incorporating a fluorescin dye in the emulsion, treating one 15 of such batch of plates to convert it to red sensitiveness by an isocyanin dye, and simultaneously exposing such converted plate and an unconverted plate from the same batch to the same light image while the two are in 20 face to face contact.

11. In the art of color photography, the process of making a plate pack comprising the following steps: producing a plurality of differently color-sensitized photographic 25 plates, coating the sensitive surface of one of them before assembling with a temporary superficial color layer suitable as a screen for one of the plates by spreading thereon a solution in alcohol and ether of dye stuff 30 and soluble cotton and assembling and securing together said plates into a plate pack.

12. In the art of color photography, the process of making a plate pack comprising 35 the following steps: producing a plurality of differently color-sensitized photographic plates, coating the sensitive surface of one of them before assembling with a temporary superficial color layer suitable as a screen 40 for one of the plates by spreading thereon a solution of substantially the proportions, alcohol 4 oz., ether 2 oz., soluble cotton 1 gr., and a suitable quantity of a dye color soluble in both alcohol and water and assembling 45 and securing together said plates into a plate pack.

13. In the art of color photography, the process of producing color-selection negatives comprising: preparing a plurality of 50 green-sensitive plates by incorporation of the color sensitizing dye or agent in the emulsion, treating one thereof with a prepotent agent capable of rendering it red-sensitive, coating a second one of such plates 55 with a temporary red color layer or screen over its sensitive face, assembling a plate-pack comprising said first plate at the rear, said second plate in front of and in face contact with the first and a blue-sensitive 60 plate in front of both, securing the whole together and simultaneously exposing them.

14. In the art of color photography, the process of making a plate-pack comprising: preparing a batch of photographic plates

sensitive to one color, coating the reverse 65 of one thereof with an opaque, water-insoluble layer, converting such reversely coated plates to sensitiveness of a different color, and assembling in face contact said converted and an unconverted plate for exposure through the support of the unconverted plate.

15. In the art of color-photography, the process of making a plate-pack comprising: preparing a batch of green-sensitive photographic plates, coating the reverse of one thereof with an opaque, water-insoluble layer, converting such reversely coated plate to red-sensitiveness, and assembling in face contact said converted and an unconverted 75 plate for exposure through the support of the unconverted plate.

16. In the art of color photography the process of producing a plate pack which comprises the following steps: coating with 85 an opaque water insoluble layer upon its reverse side one of a batch of photographic plates which have been previously green sensitized, treating said plate to convert it to red sensitiveness, assembling said plate 90 in face contact with an unconverted plate from the same batch and applying a temporary superficial color screen upon the sensitive coating of one of said plates before assemblage.

17. In the art of color photography the process of producing a plate pack which comprises the following steps: coating with 95 an opaque water insoluble layer upon its reverse side one of a batch of photographic plates which have been previously green sensitized, treating said plate to convert it to red sensitiveness, assembling said plate 100 in face contact with an unconverted plate from the same batch and applying a temporary superficial color screen upon the sensitive coating of one of said plates before assemblage; said opaque layer consisting of a mixture of asphaltum and an oil-soluble dye absorptive of red light.

18. In the art of color-photography, the process of producing color-selection negatives comprising: preparing two green-sensitive plates by incorporation of the color-sensitizing agent in the emulsion, coating 115 the first one thereof with an insoluble opaque coating over its back, treating the same thereafter with a prepotent agent capable of rendering it red-sensitive, introducing between said two plates a temporary red color layer or screen, assembling a plate-pack comprising said first plate at the rear, and the other plate at the front of and in face contact with the first, securing the assembled plates together, and simultaneously 120 exposing them.

19. In the art of color-photography, the process of producing color-selection nega-

- tives comprising: preparing two green-sensitive plates by incorporation of a green sensitizing fluorescin dye in the emulsion, coating the first one thereof with an insoluble opaque coating over its back, treating the same thereafter with an isocyanin dye for rendering it red sensitive, introducing between said two plates a temporary red color layer or screen, assembling a plate-pack comprising said first plate at the rear, and the other plate at the front of and in face contact with the first, securing the assembled plates together and simultaneously exposing them.
- 15 20. In the art of color-photography, the process of producing color-selection negatives comprising: preparing a plurality of green-sensitive plates by incorporation of the color agent in the emulsion, coating one thereof with an insoluble opaque coating over its back, treating the same thereafter with a prepotent agent capable of converting it from green-sensitive to red-sensitive, coating a second one of such plates with a
- 20 25 temporary red color layer or screen over its sensitive face, assembling a plate-pack comprising said first plate at the rear, said second plate in front of and in face contact with the first and a blue-sensitive plate in front of both, securing the assembled plates together and simultaneously exposing them.
- 25 30 35 21. A plate-pack or plate-set for color photography comprising a plurality of differently color sensitized photographic plates secured together for simultaneous exposure, two of said plates being from the same batch of color-sensitized plates, and one of said

two plates having been converted to a different color sensitiveness.

22. A plate-pack or plate-set for color 40 photography comprising a plurality of differently color sensitized photographic plates secured together for simultaneous exposure, two of said plates being from the same batch of green-sensitized plates, and one of said 45 two plates having been converted to a red-sensitiveness, and a third plate being blue-sensitive.

23. A plate-pack or plate-set for color 50 photography comprising a plurality of differently color sensitized photographic plates secured together for simultaneous exposure, two of said plates being from the same batch of color-sensitized plates, and one of said 55 two plates having been converted to a different color sensitiveness, and suitable color-selective screens located between the sensitive layers.

24. A plate-pack or plate-set for color 60 photography comprising a plurality of differently color sensitized photographic plates secured together for simultaneous exposure, two of said plates being from the same batch of green-sensitized plates, and one of said 65 two plates having been converted to a red-sensitiveness, and a third plate being blue-sensitive, and suitable color-selective screens located between the sensitive layers.

In testimony whereof I affix my signature in presence of two witnesses.

FREDERIC E. IVES.

Witnesses:

WILLIAM J. DOLAN,  
DONALD CAMPBELL.